

## UNITED STATES PATENT OFFICE

2,172,447

## INCREASING THE REACTIVITY OF CELLULOSE TO ESTERIFICATION REAGENTS

Arnold Marschall, Freiburg-in-Breisgau, Germany, assignor to E. I. du Pont de Nemours &amp; Company, Wilmington, Del., a corporation of Delaware

No Drawing. Application January 27, 1938,  
Serial No. 187,178

12 Claims. (Cl. 260—229)

This invention relates to cellulosic material and process of producing same; more particularly, it relates to a process for the treatment of cellulose with a salt whereby to greatly increase the reactivity of the cellulose to a subsequent acetylation or esterification reaction.

The various forms of cellulose which are available commercially have varying degrees of chemical reactivity, depending, among other factors, on whether the source of the cellulose is cotton, cotton linters, wood pulp, wood chips, sisal, bagasse, and the like, and in accordance with the method by which the cellulose has been purified, and the extent of the purification treatment. Thus, cellulose derived from wood pulp is generally more difficult to esterify than cellulose derived from cotton or cotton linters.

It is therefore an object of the present invention to influence and control the esterifying reactivity of cellulose, particularly cellulose which has a low chemical reactivity and is therefore difficult to esterify by previously known esterification processes.

Another object of the present invention is to provide a process for the treatment of cellulose whereby to insure a more rapid and more uniform penetration of the cellulose by the esterification reagents.

A still further object of the present invention is to provide a method for the treatment of cellulose whereby to prepare a good quality of cellulose acetate, or other cellulose derivative, from cellulose derived from wood pulp.

The above objects may be accomplished, in general, by treating cellulose with a small quantity of a water-soluble, inorganic neutral salt taken from the group consisting of sodium, potassium, lithium, ammonium, amine, and substituted amine salts of an acid taken from the group consisting of sulfuric, hydrochloric, perchloric, phosphoric, and similar strong inorganic acids. The treatment of the cellulosic material by the above-described salts is carried out prior to the treatment of the cellulose with any of the usual esterifying agents, or agents especially preparing the cellulose for esterification, such as acetic anhydride, acetic acid, sulfuric acid or the like. The salts of the present invention with which the cellulosic material is to be treated have little, if any, swelling action on the cellulose.

In accordance with the process of the present invention the treatment of the cellulosic material is preferably carried out while the cellulose is still in a completely open and swollen condition from its manufacture. By so proceeding, the cellulose

fibers will be uniformly impregnated with the salt substantially throughout their structure. To this end the application of the salt may conveniently be made a part, or a continuation, of the final washing step in the customary methods of manufacturing cellulose. The cellulosic material is preferably treated with an aqueous solution of the salt in such concentration that the salt will be present in a quantity of 0.1 to 3% based on the dry weight of the cellulose. The cellulosic material impregnated with the salt, before esterification, is preferably dried to a moisture content of less than 12%, based on the weight of the dry cellulose. The drying may be carried out by any suitable, known drying method which will not remove the salt.

Of the numerous possible salt treatments, two examples will be set forth illustrating, in detail, the process of the invention. It is, of course, to be understood that the invention is not to be limited by the examples.

## Example 1

Seventy-five kilograms of sulfite wood pulp cellulose is continuously agitated with a solution of 10 kilograms of ammonium perchlorate dissolved in 600 liters of water for a suitable period of time, after which the liquid is pressed or centrifuged off and the wood pulp dried. The dried wood pulp has 1.3 to 2.0% of ammonium perchlorate uniformly distributed and deeply embedded throughout the cellulose fibers. After acetylation by a conventional acetylation procedure, for example, the procedure described in U. S. No. 1,543,310, the ammonium perchlorate impregnated pulp surprisingly yields a cellulose acetate exhibiting the following improvement over the cellulose acetate derived by the same acetylation procedure from the same pulp without the salt pretreatment:

|                                                                                  | Pre-treated<br>pulp | Un-<br>treated<br>pulp | 40 |
|----------------------------------------------------------------------------------|---------------------|------------------------|----|
| Time of acetylation in minutes                                                   | 87                  | 135                    |    |
| Clarity: comparative transparency<br>of a layer of the acetylated solution in cm |                     |                        | 45 |
| Filterability in cc. per unit of<br>time                                         | 205                 | 139                    |    |
| Viscosity—(of a 7% acetone solution at 15° C. in c. g. s. units)                 | 288                 | 87                     |    |
|                                                                                  | 7.7                 | 7.9                    | 50 |

## Example 2

Wood pulp cellulose, prepared according to standard practice, and while still somewhat wet, and swollen from the customary washing, is

mixed with a solution of 15 kilograms of ammonium sulfate dissolved in 600 liters of water for a suitable period of time, after which the liquid is pressed or centrifuged off. After air drying, the wood pulp exhibits a salt content of 5 1.5-2.1% ammonium sulfate uniformly distributed throughout the fibers, including the interiors thereof. Upon acetylation by any standard procedure, the ammonium sulfate impregnated wood 10 pulp acetylates quite rapidly to a cellulose acetate superior in clarity and filterability to the cellulose acetate derived by the same acetylation procedure from the same pulp without the salt pretreatment.

15 Among the salts which may be used, in accordance with the present invention, for the pre-treatment of cellulosic material, the pentavalent nitrogen-containing salts of hydrochloric, sulfuric, phosphoric and perchloric acids have been 20 found to be particularly useful. Particularly good results have been obtained with ammonium chloride, ammonium phosphate, trimethylamine hydrochloride, triethylamine hydrochloride, triethylamine perchlorate, triethanolamine perchlorate, triethanolamine hydrochloride, tetra-25 methyl ammonium chloride, tetraethyl ammonium chloride, and tetraethyl ammonium perchlorate. Certain alkaline salts of the above mentioned acids have also given very useful results, for example sodium chloride, potassium chloride, sodium sulfate, potassium perchlorate, etc. The present invention does not comprehend 30 the use of salts having substantial swelling action on cellulose under normal conditions.

35 The esterification of the salt impregnated cellulose may be conducted in accordance with practically any of the known esterification methods. Thus, the esterification may be performed in such a manner that the resulting cellulose ester 40 dissolves or disperses to form a dope or, if desired, in such a fashion in the presence of a cellulose ester nonsolvent that the resulting cellulose ester retains the fibrous form of the original cellulose. If desired, instead of cellulose acetate, the esterification 45 of such pretreated cellulose may be directed to the preparation of other simple and mixed organic esters of cellulose, such as cellulose formate, cellulose propionate, cellulose butyrate, cellulose acetopropionate, cellulose aceto-50 butyrate, cellulose acetate succinate, cellulose acetate phthalate, and cellulose acetate stearate.

55 The process of the invention increases the chemical reactivity of the cellulose and makes available for esterification certain commercially occurring low grade celluloses previously generally considered unsuitable because of their known resistance toward esterification. The pretreatment appears also to permit the esterifying reagents, such as acetic acid, acetic anhydride, and sulfuric acid, to penetrate more uniformly and rapidly 60 into the interiors of the cellulose fibers, and results in a more rapid esterification. The cellulose, pretreated by the process of the invention, seemingly yields upon esterification a cellulose ester of 65 more uniform quality than normally, judging by the superior clarity and filterability exhibited. Such uniformity arises, it is believed, from the salts being uniformly and deeply distributed in the fiber interior by the salt solution treatment 70 and from the salts being embedded in the fibers by drying before subjecting the fibers to esterifying reagents. The cellulose esters may, of course, be converted by usual methods into useful structures, such as threads, films, lacquers, and 75 plastics.

Since it is obvious that many changes and modifications of the above described processes can be made without departing from the nature and spirit of the invention, it is to be understood that the invention is not to be limited except as set forth in the appended claims.

I claim:

1. The process of increasing the reactivity of cellulose to esterification reagents which comprises the step of treating the cellulose, prior to 10 its treatment with any esterification reagent, with a solution of a salt taken from the group consisting of sodium, potassium, lithium, ammonium, amine, and substituted amine salts of an acid taken from the group consisting of sulfuric, hydrochloric, perchloric and phosphoric acids, and drying the cellulose, impregnated with the salt, to a moisture content of less than 12%, 15 based on the weight of the dry cellulose.

2. The process of increasing the reactivity of 20 cellulose to esterification reagents which comprises the step of treating the cellulose, prior to its treatment with any esterification reagent, with an aqueous solution of a salt taken from the group consisting of sodium, potassium, lithium, 25 ammonium, amine, and substituted amine salts of an acid taken from the group consisting of sulfuric, hydrochloric, perchloric and phosphoric acids, and drying the cellulose, impregnated with the salt, to a moisture content of less than 12%, 30 based on the weight of the dry cellulose.

3. The process of increasing the reactivity of cellulose to esterification reagents which comprises the step of treating the cellulose, prior to 35 its treatment with any esterification reagent, with a solution of a water-soluble, pentavalent nitrogen-containing salt, and drying the cellulose, impregnated with the salt, to a moisture content of less than 12%, based on the weight of the dry cellulose.

4. The process of increasing the reactivity of 40 cellulose to esterification reagents which comprises the step of treating the cellulose, prior to its treatment with any esterification reagent, with an aqueous solution of a water-soluble, 45 pentavalent nitrogen-containing salt, and drying the cellulose, impregnated with the salt, to a moisture content of less than 12%, based on the weight of the dry cellulose.

5. The process of increasing the reactivity of 50 cellulose to esterification reagents which comprises the step of treating the cellulose, prior to its treatment with any esterification reagent, with a solution of a water-soluble, pentavalent nitrogen-containing salt in such concentration as to 55 impart to the cellulosic material 0.1 to 3% salt, based on the weight of the cellulose, and drying the cellulose, impregnated with the salt, to a moisture content of less than 12%, based on the weight of the dry cellulose.

6. The process of increasing the reactivity of 60 cellulose to esterification reagents which comprises the step of treating the cellulose, prior to its treatment with any esterification reagent, and while the cellulose is in an open or swollen condition, with a solution of a water-soluble, pentavalent nitrogen-containing salt, and drying the cellulose, impregnated with the salt, to a moisture content of less than 12%, based on the weight of the dry cellulose.

7. The process of increasing the reactivity of 70 cellulose to esterification reagents which comprises the step of treating the cellulose, prior to its treatment with any esterification reagent, with a solution of triethanolamine perchlorate. 75

8. Cellulose, having a moisture content of less than 12%, based on the weight of the dry cellulose, and having an increased reactivity to esterification reagents, containing a salt taken from the group consisting of sodium, potassium, lithium, ammonium, amine and substituted amine salts of an acid taken from the group consisting of sulfuric, hydrochloric, perchloric and phosphoric acids.
- 5 9. Cellulose, having a moisture content of less than 12%, based on the weight of the dry cellulose, and having an increased reactivity to esterification reagents, containing 0.1 to 3% of a salt taken from the group consisting of sodium, potassium, lithium, ammonium, amine, and substituted amine salts of an acid taken from the group
- consisting of sulfuric, hydrochloric, perchloric and phosphoric acids.
10. Cellulose, having a moisture content of less than 12%, based on the weight of the dry cellulose, and having an increased reactivity to esterification reagents, containing a water-soluble, 5 pentavalent nitrogen-containing salt.
11. Cellulose, having a moisture content of less than 12%, based on the weight of the dry cellulose, and having an increased reactivity to esterification reagents, containing 0.1 to 3% of a water- 10 soluble, pentavalent nitrogen-containing salt.
12. Cellulose, having an increased reactivity to esterification reagents, containing triethanol-amine perchlorate.

ARNOLD MARSCHALL. 15